

## UNITED STATES PATENT OFFICE

2,218,335

## BINDER COMPOSITION

Earl George Kerr, Cliffside Park, N. J., assignor  
to The Barrett Company, New York, N. Y., a  
corporation of New Jersey

No Drawing Application March 2, 1937,  
Serial No. 128,634

9 Claims. (Cl. 260—28)

This invention relates to binder compositions and more particularly to binders employed in the manufacture of tile used in construction of floors, walls, roofs, etc., and to the resultant tile product.

5 In the manufacture of tile, binders such as asphalt or blends of paracoumarone or related resins and stearine pitch are mixed with suitable fillers such, for example, as wood flour, asbestos fiber, other fibrous material, clay, or other inert 10 material and the mixture moulded to shape to produce the desired product. Blends of paracoumarone resin and stearine pitch have found wide application for this purpose because such blends have the necessary adhesive properties 15 and result in tile having physical properties and ageing characteristics which, while not altogether satisfactory, are as good as or better than those of tile made with other binders hitherto practically available. Stearine pitch, however, is 20 subject to oxidation on exposure to air, and tile containing it tend to become brittle and frequently shrink or warp on storage owing to oxidation of the stearine pitch.

It is an object of this invention to provide a 25 binder particularly adapted for use in the manufacture of tile, which binder will not readily oxidize on exposure to air and which possesses other desirable properties rendering it admirably suited for such use. Other objects and advantages of this invention will be made evident as 30 the description of the invention progresses.

I have discovered that pine fatty acid pitch blended with paracoumarone resin in suitable proportions gives a binder which is eminently 35 satisfactory for use in tile manufacture. This binder is not readily oxidized as is the case with binders heretofore used and with which I am familiar, and has the necessary adhesive and elastic properties which render it particularly useful 40 in the manufacture of tile. Moreover, I have discovered that pine fatty acid pitches soften and toughen paracoumarone resin without greatly increasing the temperature susceptibility of the resultant blended binder, i. e., the melting point 45 of the resultant composite binder will not be reduced to a point where the binder bleeds or softens when subjected to temperatures normally encountered by the finished tile in use. As compared with paracoumarone resin alone, the composite binder improves the toughness and reduces the brittleness of the tile, even at the lowest temperatures encountered in normal use thereof. A further advantage of pine fatty acid pitch over other materials heretofore commonly 50 blended with paracoumarone or similar resins

is that it fluxes more readily with such of these resins as are difficultly soluble in oils. Hence, the use of pine fatty acid pitch results in a more homogeneous binder. The binder of this invention results in a tile which weathers better owing 5 to the less brittle characteristics thereof and to its greater resistance to oxidation, with consequent less likelihood of the tile being broken or chipped in application and use than time made with other binders such as the paracoumarone-resin-stearine-pitch binder heretofore commonly used.

I have made the further surprising discovery 10 as a result of extensive experimental work in developing my invention, that it is not necessary to replace all of the stearine pitch of previous formulas with pine fatty acid pitch in order to obtain the beneficial results of the latter. For example, a binder containing 40% stearine pitch and no pine fatty acid pitch was found unsatisfactory, whereas by replacing 15 parts of the 40 parts of the stearine pitch with pine fatty acid pitch, a satisfactory binder resulted, i. e., tiles made with it did not warp or shrink. One possible explanation of this surprising result which 15 occurs to me, based on the work I have done in this field, is that the pine fatty acid pitch contains a protective agent or anti-oxidant which prevents or sufficiently minimizes deleterious 20 oxidation of the stearine pitch to yield a satisfactory 25 binder.

Pine wood fatty acid pitch may be obtained by 30 working up the resinous material removed from pine wood in the manufacture of paper or pulp in accordance with well-known procedures practiced in making paper from such wood. This resinous material is distilled, under vacuum and with the aid of steam if desired, to remove distillates including abietic acid rosin, leaving a 35 residue of pine fatty acid pitch which is employed 40 in the manufacture of the binder of this invention. The melting point of the pine fatty acid pitch used may fall within the range of about 70° to 140° F.; preferably a pitch having a melting 45 point of about 100° F. is used.

A minor amount of the pine fatty acid pitch is 50 blended with a major amount of the paracoumarone resin having a melting point of from about 194° to 320° F., preferably about 250° F. in the proportion of from 50% to 80% resin to 50% to 20% pine fatty acid pitch, the resultant binder 55 mixed with the filler and the mixture moulded to produce the desired hard tile product. Preferably the blending is accomplished by melting the paracoumarone resin by heating it and then 60

adding the pine fatty acid pitch to the melted resin as fast as it dissolves therein. In one example of making the binder of this invention in this manner 66½% of paracoumarone resin of 245° F. melting point was blended with 33½% pine fatty acid pitch of about 122° F. melting point to produce an eminently satisfactory tile binder of 187° F. melting point.

Paracoumarone resin is ordinarily made by the 10 sulfuric-acid polymerization of coal tar or water gas tar naphtha fractions containing coumarone, indene and associated polymerizable compounds. Other polymerization methods may be used. Naphthas from cracked gasoline or from 15 polymerized natural or petroleum-refinery gases may be similarly treated to yield resins. I refer to these resins collectively as "naphtha resins."

Part or all of the ordinary paracoumarone 20 resin used in my product may be replaced by other naphtha resins, and, as above indicated, a mixture of stearine and pine fatty acid pitches may be used instead of the latter alone; e. g., in ratios of pine fatty acid pitch to stearine pitch 25 of 1:3 and upwards, i. e., the amount of pine fatty acid pitch being equal to at least ⅓ of the amount of stearine pitch.

An example of a satisfactory binder containing both stearine and pine fatty acid pitches 30 follows:

| Per cent                                        |
|-------------------------------------------------|
| Paracoumarone resin, melting point 245° F. 60   |
| Pine fatty acid pitch, melting point 105° F. 15 |
| Stearine pitch, 147° F. 25                      |

35 Melting point of binder, 196° F.

Tile made with the binder of this invention may contain about 30% binder and 70% filler material which may be constituted of

| Per cent                                           |
|----------------------------------------------------|
| 40 Long fibered asbestos 20                        |
| Short fibered asbestos 35                          |
| Finely divided (air floated) silica 10             |
| Pigment, e. g. red oxide of iron for a red tile. 5 |

45 The percentage figures in the above table are in terms of per cent of each of the filler constituents based on the total constituents of the tile. The above data represent a typical formula for a tile containing the binder of this invention and, it will be understood, considerable variation in the proportions is permissible. For example, from 25 to 35% binder may be used; the amount of long fibered asbestos may be reduced to 15% and in some cases to as low as 10%. The 50 long fibered asbestos is a strength-imparting constituent, and since it is considerably more expensive than the other constituents, the amount thereof is kept as low as possible compatible with a satisfactory tile. The silica acts to fill the in-

terstices in the fibrous portion of the filler and has a beneficial effect when the mixture is milled in that it aids in the elimination of air from the mix and consequently avoids formation of blisters in the final product.

The pigment and fibrous material may be added to the binder in a suitable mixer in which heat is maintained and the mixing continued until a tough homogeneous plastic mass is obtained. From the mixing machine the plastic mass is fed between a pair of milling rolls where the mix is milled to remove blisters therefrom. From the milling rolls the mass in sheet form is fed through calendar rolls where it is reduced to the desired thickness. The resultant sheet is 15 then fed through dieing equipment where tiles of the desired shape are produced.

It is to be understood this invention is not restricted to the present disclosure otherwise than defined by the appended claims.

What is claimed is:

1. A homogeneous composition suitable for use as a binder comprising pine fatty acid pitch and naphtha resin.

2. A homogeneous binder suitable for use in 25 the manufacture of tile comprising pine fatty acid pitch blended with paracoumarone resin.

3. A homogeneous binder suitable for use in the manufacture of tile consisting of pine fatty acid pitch blended with paracoumarone resin.

4. A homogeneous binder suitable for use in 30 the manufacture of tile comprising 20% to 50% of pine fatty acid pitch blended with 80% to 50% naphtha resin.

5. A homogeneous binder suitable for use in 35 the manufacture of tile comprising 80% to 50% paracoumarone resin having a melting point of from 194° to 320° F., blended with 20% to 50% pine fatty acid pitch having a melting point of from 70° to 140° F.

6. A homogeneous binder suitable for use in 40 the manufacture of tile consisting of about 33½% pine fatty acid pitch having a melting point of about 122° F. blended with about 66½% paracoumarone resin having a melting point of about 245° F.

7. A tile comprising filler material and a binder 45 comprising pine fatty acid pitch blended with naphtha resin.

8. A tile comprising filler material and a binder 50 comprising a major amount of paracoumarone resin having a melting point of from 194° to 320° F. and a minor amount of pine fatty acid pitch having a melting point of from 70° to 140° F.

9. A homogeneous binder composition suitable 55 for use in the manufacture of floor tile comprising a blend of paracoumarone resin, pine fatty acid pitch and stearine pitch.

EARL GEORGE KERR.